

# UNITED STATES PATENT OFFICE.

CHARLES A. BROWN, ELIAS B. DENISON, AND CHARLES D. BROWN, OF  
PORTLAND, MAINE.

## BOX-BOARD.

SPECIFICATION forming part of Letters Patent No. 289,383, dated December 4, 1883.

Application filed August 6, 1883. (No specimens.)

*To all whom it may concern:*

Be it known that we, CHARLES A. BROWN, ELIAS B. DENISON, and CHARLES D. BROWN, of Portland, in the State of Maine, have invented a new and useful Improvement in Box-Board made from pulp obtained from grinding wood.

It is important that box-board should be cheaply made; that it should be of a light color and possess considerable strength. Wood pulp made by simply grinding the wood will produce a board of nearly the same color as the wood itself, and therefore by using wood of a light color pulp may be obtained of a desirable color for box-board. It will, however, if made from the varieties of wood usually employed, lack the strength which is desirable.

It is well known that if wood is steamed or boiled for a considerable time before it is ground a pulp is obtained without much increase in expense which will make a much stronger board, but of a darker color, than that obtained from wood of the same kind not so treated.

To secure a gain in strength without the dark color and without much increase in cost is the object of our invention. We secure these results by combining in the process of making the board one or more layers of dark pulp from steamed or boiled wood with one or more layers of light-colored unsteamed or unboiled wood, the latter giving a surface of

desirable color, while the former gives a greater degree of strength than has heretofore been secured from ordinary ground pulp alone not 31 boiled or steamed. These layers are produced from the pulp and combined together in the ordinary manner of forming thick paper or board by combining different layers of moist pulp into one sheet, as upon a so-called "cylinder-machine." Where both sides are to be 40 of light color, the layer of steamed or boiled pulp will be laid between the layers of light color; but if only one surface is to be of light color the other surface will be made by a layer 45 of the steamed or boiled pulp.

We are aware that paper has been made with a surface of manila applied to a body of ground wood pulp, and of ordinary coarse and dark straw pulp with a surface of ground wood 50 pulp; and also of bleached manila pulp combined with unbleached manila pulp.

We claim—

Box-board made from ground wood pulp, steamed or boiled, with ground wood pulp unsteamed applied to its surface, substantially 55 as described.

CHAS. A. BROWN.  
ELIAS B. DENISON.  
CHARLES D. BROWN.

Witnesses:

FRANKLIN C. PAYSON,  
HENRY S. PAYSON.